

Aug. 30, 1949.

A. E. MATSON ET AL

2,480,156

ELECTRODEPOSITION OF IRON

Filed Nov. 24, 1944

2 Sheets-Sheet 1



INVENTORS  
Amel E. Matson  
Harold V. Trask  
BY John E. Thygesen Jr.  
ATTORNEY

Aug. 30, 1949.

A. E. MATSON ET AL

2,480,156

## ELECTRODEPOSITION OF IRON

Filed Nov. 24, 1944

2 Sheets-Sheet 2

75. Fig. 3



*INVENTORS*

INVENTORS  
Amel E. Matson  
Harold V. Trask  
BY John E. Thyber Jr.  
ATTORNEY

## UNITED STATES PATENT OFFICE

2,480,156

## ELECTRODEPOSITION OF IRON

Amel E. Matson and Harold V. Trask, Nashwauk,  
Minn., assignors to Euel Metals Company, St.  
Paul, Minn., a corporation of Ohio

Application November 24, 1944, Serial No. 564,935

6 Claims. (Cl. 204—10)

1

This invention relates to the production of a pure, brittle iron suitable for use in powder metallurgy and particularly to an electrolytic process for producing iron of such brittle character that it may be readily pulverized to particles of the required sizes and of such dendritic or angular structure as to cause them to intermesh with each other uniformly in the forming dies.

It is an object of our invention to provide a novel and economical method for producing such iron by electrodeposition.

Another object is to provide a process of this general character which includes steps for continuously reconditioning the electrolyte with respect to its ferrous and ferric iron content, as well as its pH and temperature in order to maintain certain critical proportions of constituents in the electrolyte and other beneficial conditions in the deposition cells.

A further and particular object is to provide a method for producing a pure, brittle iron by two stages of electrodeposition in the first stage of which anodes for use in the second stage are produced and wherein the necessary concentrations of ferrous and ferric salts in the electrolyte for the second stage are produced in the cell or cells of the first stage.

Other objects will appear and be more fully pointed out in the following specification and claims.

Electrodeposited iron as ordinarily produced is too malleable to permit economical grinding or other pulverization and when ground a large proportion of the particles have had such flat structures that they tend to stratify in the forming dies with the result that the products formed from the iron powder have had an irregularly laminated and relatively weak structure. Our improved iron is sufficiently brittle, having hardness equal to from 400 to 500 diamond scale, as deposited at the cathodes to permit economical crushing. It contains hydrogen and oxygen in amounts which when added together equal less than 1% of the total weight of deposit and less than one-half of 1% of other impurities. We crush our brittle deposit in a ball mill or other suitable grinding machine to particles of the desired size (usually minus 100 mesh) and then drive off the hydrogen and oxygen by simple annealing treatment in a reducing atmosphere and at temperatures so low that only slight fritting of the particles results. This produces a powder which is more than 99.5% pure iron and in which the desired structure of the particles is retained. In some cases a secondary pulverizing treatment may

2

be necessary to separate the individual particles after the annealing treatment.

Our process may be carried out in open cells without diaphragms between the anodes and cathodes. As the source of the iron, ingot iron plates of suitable thickness, preferably about one inch thick, may be used. These plates may contain up to .2% of carbon and substantial amounts of other impurities. For example, the anode plates may contain .03% carbon, and manganese, silicon, phosphorous and sulphur totaling together approximately .10% and copper approximately .15%.

Instead of using ingot iron plates as the anodes, according to our invention the anodes may be produced by electrodeposition carried out in separate cells concurrently with the electrolysis in the cells producing the brittle deposit. A separate deposition chamber wherein the anodes are insoluble may also be used as a continuous source of ferric iron to be introduced into the electrolyte of the main deposition chamber, as more fully hereinafter described.

Our cathode starting sheets in the main or secondary deposition chambers are of such flexible character that the brittle deposit may be removed therefrom periodically by flexing. We prefer to use stainless steel cathode sheets having the desired flexibility in the main deposition chambers

and mild steel sheets to start the cathodes in the primary deposition chambers. Stainless steel sheets containing 18% chromium and 8% nickel and of 16-gauge thickness have been found to be adequately stiff to remain straight in the cells while affording the flexibility necessary to permit ready removal of the iron deposit by flexing. The mild steel cathode starting sheets may contain carbon up to .2% and other impurities as in the case of the ingot iron plate for use as soluble anodes in the main deposition chamber.

Our electrolyte may be produced by dissolving scrap iron of low carbon content in hydrochloric acid. The concentrated solution of ferrous chloride is preferably diluted so that it contains from 150 to 250 grams of iron per liter of solution. For use in the main deposition chamber where the brittle iron is deposited the electrolyte must contain from 1 to 5 grams of iron as ferric iron per liter of solution and its pH must be maintained below 1.2 and preferably from 1 to 1.1 by the addition of a sufficient quantity of hydrochloric acid.

Another important factor in obtaining a brittle deposit of pure iron at the cathodes is the control of the temperature in the cell so that it does not exceed 50 degrees C., and is preferably maintained

between 20 and 30 degrees C. The temperature may be regulated by continuously circulating the electrolyte through a heat exchanger or otherwise by cooling the walls of the deposition chambers. The use of a heat exchanger located exteriorly of the cell is preferred since it is desirable to maintain the electrolyte in circulation through the cells and this may be accomplished economically by the use of a pump and conduits arranged to continuously withdraw the electrolyte from one end of the cell and to return it to the opposite end after it has been subjected to conditioning treatment, as required. A filter is used in the circuit to remove any solid impurities that may be derived from the impure anodes or other source of iron such as the scrap iron contained in the leach tanks.

In subjecting an electrolyte of the character described to electrolysis for our purposes, it is further important that the rate of flow of current between the electrodes be maintained at a current density of over 25 amperes per square foot and preferably at 30 amperes per square foot. This is a contributing factor in producing a brittle deposit of iron and has the further effect of reducing the power consumption and generally increasing the efficiency of the process.

Referring to the drawings which illustrate diagrammatically suitable flow sheets and apparatus for carrying out our invention:

Figure 1 shows one arrangement of electrolytic cell in electric circuit with a source of direct current and including connections with suitable apparatus for conditioning the electrolyte;

Fig. 2 illustrates a specific procedure wherein primary and secondary deposition cells are employed and the ferric chloride is supplied from the primary cell, and

Fig. 3 illustrates another arrangement of apparatus and procedure wherein the anodes for use in the main cell or cells are produced by electro-deposition in auxiliary cells.

Referring to Fig. 1, the numeral 2 indicates a tank constituting the deposition chamber or cell which may be constructed of suitable material such as rubber, acid-resisting brick, or other material capable of withstanding the corrosive action of the electrolyte contained in the tank. The electrodes comprise a multiplicity of iron anode plates 3 and cathode sheets 4 shown in groups in the tank 2. The cathode sheets extend in suitably spaced, parallel and intermeshing relation to the anode plates of each group, being submerged in an electrolyte of the character hereinbefore described within the tank 2. A source of direct current, indicated by the numeral 5, is connected in circuit with the electrodes by means of conductor cables 6 and 7 extending to bus bars 8 and 9 respectively. As shown, individual plate connectors 8a extend from the bus bars 8 to the several anode plates 3 of the first group, the cathode sheets 4 of which have connectors 10a extending to a bus bar 10. Similar connectors 10b connect the anode plates 3 of the second group to the bus bar 10. The cathode sheets of the second group are in circuit through individual connectors 11a with a bus bar 11 and similar connectors 11b extend from bar 11 to the several anode plates of the third group. In a like manner the cathode sheets of the third group are connected to the anode plates of the fourth group through a bus bar 12 and connectors 12a and 12b while the several cathode sheets of the fourth group have connectors 9a extending to the bus bar 9. It will thus be evident that the several

groups of electrodes are connected in series so that an electric current may be caused to flow from the source 5 between the several cathodes and anodes and intervening electrolyte. When the current is caused to flow through this circuit iron is deposited by electrolysis on the cathodes as it is dissolved from the anodes in a manner well known in the art.

As further indicated in Fig. 1, the electrolyte is continuously circulated through the deposition chamber comprising the tank 2 and is reconditioned and then returned for further electrolysis. A pipe 13 conducts the electrolyte from one end of the tank 2 to a pump 14 which is power driven to maintain circulation at the desired rate of flow through the apparatus and conduits presently to be described. From the outlet of the pump a pipe 15 extends to a filter 16 from which a pipe 17 extends to a heat exchanger 18 having coils wherein the electrolyte is cooled. A cooling medium is supplied to the heat exchanger 18 through an inlet pipe 19 and is discharged through a pipe 20. From the heat exchanger the electrolyte is returned to the tank 2 through a pipe 21.

A branch 22 of the pipe 21 extends to a source 23 of ferric chloride solution and the flow of this solution to the pipe 21 is under control of a valve 24. Another branch 25 of the pipe 21 supplies hydrochloric acid from a source 26 and the pH of the electrolyte is controlled by adjustment of a valve 27 in the pipe 25. It is necessary to add only a small amount of free acid to the electrolyte to maintain its pH below 1.2 because the desired hydrogen ion concentration is made up in part by the addition of ferric chloride to the electrolyte in an amount equal to less than five grams of ferric iron per liter of solution. By this conditioning treatment for the electrolyte and by causing current to flow from the source 5 to a density between electrodes of approximately 30 amperes per square foot, we maintain conditions in the deposition chamber which are favorable to a brittle deposit on the cathode sheets 4.

In operation, from time to time as iron is deposited on the stainless steel cathode sheets 4 these sheets are removed from the cell and flexed to dislodge the relatively brittle deposit, after which they may be replaced in the tank to receive a further deposit of pure iron. Separation of the brittle iron coating from the cathode sheets is facilitated if the coating is not allowed to exceed about  $\frac{5}{32}$  inch in thickness. The flexing of the iron coated sheets may be performed manually by bending the sheets over a roller or bar or otherwise in a machine designed for the purpose. After repeated use it is sometimes necessary to clean the cathode sheets before returning them to the tank and this may be accomplished by dipping them in dilute hydrochloric acid for a period of from one to five minutes. Cathode sheets of the character described are so durable that they may be used according to our invention almost indefinitely. It will be evident that the anode plates must be replaced by new ones periodically as they are dissolved in the electrolyte.

In Fig. 2 the main deposition cell is indicated by the numeral 28, the anode plates by the numeral 29 and the cathode starting sheets by the numeral 30. Conditions in the cell 28 with respect to temperature, current density, pH of electrolyte and concentration of ferric and ferrous salts in the electrolyte are maintained as hereinbefore described with reference to Fig. 1 75 in order to obtain a pure, readily grindable de-

posit on the cathode sheets 30. As further indicated in Fig. 2, we provide an auxiliary deposition chamber comprising a cell 31 in which are mounted insoluble anode plates 32 and mild steel or sheet iron cathodes sheets 33. A source 34 of direct current is connected to bus bars 35 and 36 by branch circuit cables 37 and 38 respectively. The several anodes 32 are connected to the bus bar 35 and the cathodes 33 are connected to a bus bar 39 which is also connected to a group of the cathodes 30 and another and separate group of the anodes 29 in the cell 28. The anodes 29 associated with the first mentioned group of cathodes 30 are connected to the bus bar 36 and the cathodes of the second group are connected to a bus bar 40 which is in circuit with a cable 41 extending to the source 34 of current. By this arrangement current is caused to flow with the desired density in the cells 28 and 31.

The electrolyte is caused to flow continuously from the cell 28 through a conduit 42 to the cell 31 and thence through a pipe 43 to a power-driven pump 44. This pump forces the electrolyte through a pipe 45 to and through a filter 46, then through a pipe 47 to a heat exchanger 48 and from the latter through a pipe 49 which returns it to the chamber 28. A small amount of hydrochloric acid is continuously fed into the pipe 49 from a tank 50 through a pipe 51 under control of a valve 52. The concentration of iron in the electrolyte, when it reaches the cell 31 is equal to approximately 200 grams of iron per liter, the greater portion of which is in the ferrous state although about one to two grams per liter remain as ferric iron. In the cell 31 containing the insoluble anodes 32 iron is deposited on the cathode sheets 33 resulting in a partial oxidation of the ferrous chloride to ferric chloride and impoverishment of the iron in solution. A sufficiently high rate of flow of electrolyte through the cell 31 is maintained to prevent "dead spots" and excessive impoverishment of the solution. For best results not more than 20 grams of iron should be removed per liter of solution. Consequently, as withdrawn from cell 31 through the pipe 43 the electrolyte should contain approximately 5 grams of ferric iron per liter of solution. It is then conducted through the filter 46 and cooler 48 and returned to the cell 28 through the pipe 49. The requisite amount of hydrochloric acid is fed into the solution through the branch pipe 51.

In the cell 28 the electrolyte is enriched by the dissolution of the anodes 29 with the result that a portion of its ferric salt content is reduced to the ferrous salt. This loss of ferric iron must be made up either by introducing a suitable solution for an external source, as indicated in Fig. 1, or by electrolysis, as in the cell 31, or in some other manner. The iron deposit on the cathodes 33 may be allowed to accumulate until these electrodes are thick enough for use as anodes in the cell 28. They may then be replaced by new mild steel or thin iron cathode starting sheets in the cell 31 and used as anodes 29 as the latter require replacement. It will be understood that the brittle deposit is removed periodically from the flexible cathode sheets 30 for use in iron powder metallurgy.

In Fig. 3 of the drawings we have shown a main deposition cell 52 and auxiliary cells 53, 54 and 55 in an arrangement whereby the anodes for the cell 52 may be formed by electrolysis in the other cells. Each of the auxiliary cells contain a group of insoluble anodes 56 and sheet 75

steel or iron cathodes 57. The main cell 52 has soluble iron anodes 58 and relatively thin, flexible cathodes 59. The electric circuit comprises a source of direct current 60 and circuit cables 61 and 62 having branches 63 and 64, extending respectively to bus bars 65 and 66 of the cell 52. A bus bar 67 for the cell 53 is connected to the cable 61 and a bus bar 68 for the cell 55 is connected to the cable 62. The cell 53 has a bus bar 69 connected in series with a bus bar 70 of the cell 54 and a bus bar 71 for the cell 54 is connected in series with a bus bar 72 for the cell 55. Individual connectors extend from the bus bar 67 to the several anodes 56 of the cell 53 and other individual connectors join the cathodes 57 of the cell 53 with the bus bar 69. In like manner, the several anodes and cathodes of the cells 54 and 55 are connected to the respective bus bars of these cells so that current may be caused to flow from the source 60 successively through cells 53, 54 and 55. The circuit including the latter is in parallel with that comprising the cables 63, cell 52 and cable 64. In the latter circuit current is caused to flow between electrodes 58 and 59 at a current density greater than 25 amperes per square foot while in the cells 53, 54 and 55 a rate of flow between electrodes may be maintained at approximately 6 to 10 amperes per square foot.

The electrolyte for the several cells 52, 53, 54 and 55 may be formed initially by dissolving scrap iron in hydrochloric acid. Provision is made for circulating the solution through these cells and through conditioning apparatus. The flow sheet shown in Fig. 3 includes leach tanks 73 and 74 containing scrap iron and from which the electrolyte is caused to flow through a pipe 75 having branches for severally supplying the cells 53, 54 and 55 at one end. From the opposite end of each of these cells the solution is conducted to a pipe 76 having a branch 77 arranged to supply a power-driven pump 78. The outlet of this pump comprises a pipe 79 extending to the leach tank 73 from which the solution flows through a pipe 80 to the tank 74. Branch pipe 77 has a valve 81 for controlling the flow of solution to the pump 78. Another branch 82 of the pipe 76 conducts a part of the electrolyte to a power-driven pump 83 under control of a valve 84. From the pump 83 electrolyte is caused to flow successively through a filter 85 and a heat exchanger 86 and then through a pipe 87 to one end of the cell 52. A branch 88 of the pipe 87 is arranged to feed hydrochloric acid into the pipe 87 from a tank 89 under control of a valve 90. The conditioned electrolyte after flowing through the cell 52 is preferably returned to the cells 53, 54 and 55 through a pipe 91 and the several branches of pipe 75. By this arrangement of conducting and conditioning apparatus we maintain conditions in the deposition cell 52 similar to those in the cell 2 of Fig. 1 and in the cell 28 of Fig. 2. The electrolyte in cell 52 contains a total of from 150 to 250 grams of iron per liter of solution of which from 1 to 5 grams are ferric iron, the temperature in this cell is kept below 50 degrees C. and the pH below 1.2. In the cells 53, 54 and 55 no control of the temperature is necessary and the pH and ferric iron content of the electrolyte are also relatively unimportant factors where a fairly pure, soft and malleable deposit is to be formed. A pH of from 1 to 3.5 is suitable.

In operation, the electrolyte as withdrawn from the cells 53, 54 and 55 through the pipe 76 con-

tains approximately 5 grams of ferric iron per liter of solution. A sufficient quantity of this electrolyte is caused to flow through the branch pipe 82 to the pump 83 which forces it continuously through the filter 85, heat exchanger 86, cell 52 and connecting pipes including pipes 91 and 75, thus returning it to the cells 53, 54 and 55. As the anodes 58 dissolve in the electrolyte, iron is deposited in a pure brittle form on the cathodes 59 and is removed therefrom periodically, as hereinbefore described. When the anodes 58 require replacement, new anodes are obtained from the cells 53, 54 and 55 where the cathode sheets 57 are allowed to increase in thickness until they are suitable for use as anodes in the cell 52. It will be evident that a proper balance between the ferric and ferrous iron content of the electrolyte is maintained by successively passing the solution through the leach tanks 73 and 74 where the ferrous iron is replenished and then through the cells 53, 54 and 55 where the oxidation to ferric iron in a controlled degree takes place.

The presence of ferric chloride in the proportion to ferrous chloride hereinbefore described creates good mechanical conditions for deposition in that it prevents the formation of trees by acting as a depolarizer with respect to hydrogen which tends to adhere to the cathode surfaces and it also assists in making a brittle deposit of the purity required. The free acid present in the electrolyte is also beneficial in that it prevents the formation of hydrolyzed iron.

In the main deposition cells containing the soluble anodes and flexible cathodes, we prefer to use anode plates of approximately one inch thickness and to space the electrodes approximately two inches, center to center, in order to obtain a voltage drop between each pair of electrodes equal to from 2 to 2.1 volts where a current density of approximately 30 amperes per square foot is required.

It is to be understood that the foregoing specific description referring to the diagrammatic illustrations of flow sheets in the several views of the drawings are given by way of illustration and not for the purpose of limiting the present invention. Other arrangements of the electrodes in the circuit will be obvious to those skilled in the art and it will also be evident that in commercial operations a large number of cells may be connected either in parallel or in series in the electric circuit and that other arrangements of conduits and conditioning apparatus may be provided within the scope of the appended claims.

A pure, brittle iron deposit may be produced according to our invention at low cost. The cost of grinding our product is also low as compared with ordinary electrodeposited iron products. Tests show that it has hardness (diamond scale) between 400 and 500 and that it may be pulverized to particles of minus 100 mesh sizes in a ball mill at the rate of approximately 10 to 15 pounds per 100 pounds of balls per hour. After the grinding and annealing treatment a major fraction equal to approximately 95% of all particles have structures of dendritic or other angular shapes adapted to interlock or intermesh with each other in the dies. This powder when cold die pressed under pressures of the order of magnitude of 30 to 50 tons per square inch forms self-sustaining bodies which may be subjected to sintering temperatures to unite the component iron particles in bodies having great and uniform strength throughout. For many purposes these bodies may be formed with such smooth surfaces

and so accurately to dimension that no machining or other finishing operation is necessary.

Having described our invention, what we claim as new and desire to protect by Letters Patent is:

1. The method of making electrodeposited iron of pure, brittle character by two stages of electrodeposition which comprises subjecting an electrolyte consisting essentially of ferrous chloride and containing from 150 to 250 grams of iron per liter of solution to electrolysis in a cell having cathodes and insoluble anodes and wherein from 2% to 10% of the iron is oxidized to ferric iron, withdrawing the electrolyte from said cell, cooling at least a portion of it, adding free acid thereto and introducing the electrolyte so conditioned into a second cell containing cathodes and soluble iron anodes produced by electrolysis in the first mentioned cell, subjecting said solution to electrolysis in the second cell to produce a brittle deposit on the cathodes therein by maintaining in the second cell an aqueous solution consisting essentially of ferric and ferrous chloride at a total concentration of 150 to 250 grams of iron per liter of solution of which from 1 to 5 grams is ferric iron, maintaining the temperature of the solution below 50 degrees C., the pH from 1 to 1.2 and the current density of deposition not less than 25 amperes per square foot, withdrawing the electrolyte from the second cell and reintroducing it into the first mentioned cell for further electrolysis therein.

2. The method of making electrodeposited iron of pure, brittle character by two stages of electrodeposition which comprises subjecting an electrolyte consisting essentially of ferrous chloride and containing from 150 to 250 grams of ferrous iron per liter of solution to electrolysis in a cell having cathodes and insoluble anodes and wherein from 2% to 10% of the iron is oxidized to ferric iron, withdrawing the electrolyte from said cell, cooling at least a portion of the electrolyte exteriorly of said cell, adding free acid thereto, introducing the so conditioned electrolyte into a second cell containing cathodes and soluble iron anodes produced by electrolysis in the first mentioned cell, subjecting said solution to electrolysis in the second cell to produce a brittle deposit on the cathodes therein by maintaining in the second cell an aqueous solution consisting essentially of ferric and ferrous chloride at a total concentration of 150 to 250 grams of iron per liter of solution of which from 1 to 5 grams is ferric iron, maintaining the temperature of the solution below 50 degrees C., the pH from 1 to 1.2 and the current density of deposition not less than 25 amperes per square foot, withdrawing the electrolyte from the second cell and reintroducing it into the first mentioned cell for further electrolysis therein, continuously withdrawing another portion of the electrolyte from the first mentioned cell and enriching its iron content and returning the enriched electrolyte to the first mentioned cell.

3. The method of making electrodeposited iron of pure, brittle character by two stages of electrodeposition which comprises subjecting an electrolyte consisting essentially of ferrous chloride and containing from 150 to 250 grams of ferrous iron per liter of solution to electrolysis in a cell having cathodes and insoluble anodes and wherein from 2% to 10% of the iron is oxidized to ferric iron, withdrawing the electrolyte from said cell, cooling at least a portion of the electrolyte exteriorly of said cell, adding free acid thereto, introducing the so conditioned electrolyte into a second cell containing cathodes and soluble iron anodes pro-

duced by electrolysis in the first mentioned cell, subjecting said solution to electrolysis in the second cell to produce a brittle deposit on the cathodes therein by maintaining in the second cell an aqueous solution consisting essentially of ferric and ferrous chloride at a total concentration of 150 to 250 grams of iron per liter of solution of which from 1 to 5 grams is ferric iron, maintaining the temperature of the solution below 50 degrees C., the pH from 1 to 1.2 and the current density of deposition not less than 25 amperes per square foot, withdrawing the electrolyte from the second cell and reintroducing it into the first mentioned cell for further electrolysis therein, continuously withdrawing another portion of the electrolyte from the first mentioned cell, enriching its iron content by passing it through a leach tank containing impure iron and returning the enriched electrolyte to the first mentioned cell.

4. The method of making a substantially pure iron powder which includes the steps of maintaining in a cell a solution containing essentially ferrous and ferric chloride and water at a total concentration of not less than 150 and not greater than 250 grams of iron per liter of solution of which from 1 to 5 grams is ferric iron, subjecting said solution to electrolysis at a current density not less than 25 amperes per square foot between a cathode and a soluble iron anode while maintaining the temperature of the solution below 50 degrees C. and the pH thereof from 1 to 1.2, to thereby produce a brittle, coherent iron deposit containing hardening oxygen and hydrogen compounds removable by annealing and less than 0.5% of other impurities, then pulverizing the brittle deposit to particles of shapes and sizes suitable for compaction in forming dies, and annealing the resulting powder in a reducing atmosphere.

5. The method of making a substantially pure iron powder which includes the steps of maintaining in a cell a solution containing essentially ferrous and ferric chloride and water at a total concentration of not less than 150 and not greater than 250 grams of iron per liter of solution of which from 1 to 5 grams is ferric iron, subjecting said solution to electrolysis at a current density not less than 25 amperes per square foot between a cathode and a soluble iron anode while maintaining the temperature of the solution below 50 degrees C. and the pH thereof from 1 to 1.2, to thereby produce a brittle iron deposit containing hardening oxygen and hydrogen compounds removable by annealing and less than 0.5% of other

impurities, then grinding the brittle deposit so formed to particles of minus 100 mesh sizes and suitable for use in powder metallurgy and annealing the powder in a reducing atmosphere and at a low fritting temperature.

5 6. The method of making a substantially pure iron powder which includes the steps of maintaining in a cell a solution containing essentially ferrous and ferric chloride and water at a total concentration of not less than 150 and not greater than 250 grams of iron per liter of solution of which from 1 to 5 grams is ferric iron, subjecting said solution to electrolysis at a current density of approximately 30 amperes per square foot between a cathode and a soluble iron anode while maintaining the temperature of the solution below 50 degrees C. and the pH thereof from 1 to 1.2, to thereby produce a brittle iron deposit containing hardening oxygen and hydrogen compounds removable by annealing and less than 0.5% of other impurities, then pulverizing the brittle deposit, and annealing the resulting powder in a reducing atmosphere to produce a powder a major fraction of the particles of which have 10 shapes adapted to intermesh when cold die 20 pressed under suitable pressure.

AMEL E. MATSON.  
HAROLD V. TRASK.

#### REFERENCES CITED

The following references are of record in the file of this patent:

#### UNITED STATES PATENTS

| Number    | Name             | Date           |
|-----------|------------------|----------------|
| 1,980,381 | Cain             | Nov. 13, 1934  |
| 2,157,699 | Hardy            | May 9, 1939    |
| 2,223,928 | Whitfield et al. | Dec. 3, 1940   |
| 2,287,082 | Bauer            | June 23, 1942  |
| 2,385,269 | Globus           | Sept. 18, 1945 |

#### FOREIGN PATENTS

| Number  | Country       | Date |
|---------|---------------|------|
| 10,655  | Great Britain | 1909 |
| 543,137 | Great Britain | 1942 |
| 549,954 | Great Britain | 1942 |
| 813,426 | France        | 1937 |

#### OTHER REFERENCES

Transactions of the Electrochemical Society, vol. 80 (1941), pages 503, 504.

Transactions of the Electrochemical Society, vol. 84 (1943), pages 305, 306, 308, 309.